

## UNITED STATES PATENT OFFICE

FREDERICK A. KORMANN, OF GLENDALE, CALIFORNIA, ASSIGNOR TO INDUSTRIAL RESEARCH LABORATORIES LTD., A CORPORATION OF NEVADA

## COPPER-LEAD ALLOY PROCESS

No Drawing.

Application filed June 6, 1932. Serial No. 615,768.

This invention relates to copper-lead alloys of high lead content and has for its object an improved process for producing such alloys, whereby the metal produced is of perfect homogeneity and may be repeatedly remelted without stratification.

The value of copper-lead alloys as a bearing metal of high anti-friction qualities has been known for many years, but on account of the difference in physical qualities of these two metals considerable difficulty has been encountered by the metallurgist in securing satisfactory alloys where the percentage of lead was over 25%, and since a permissible lead content for average bearing unit pressures may be around 40% and in anti-friction packing glands even as high as 90%, many attempts have been made to combine these metals with the aid of various fluxing materials in order to achieve the desired end of a high lead content, but to date there is no satisfactory high lead content copper-lead alloy available on the market which can be depended upon to remain homogeneous under the various conditions of use.

In working on the problem I have found that these metals may be made to alloy perfectly in almost any proportion by incorporating a small quantity of beryllium oxide to the melt.

In carrying out the process I may place the desired quantities of the metals in a crucible together with a small quantity of beryllium oxide and cover the top with charcoal to prevent oxidation, or the copper may be melted first, the beryllium and lead added. When molten, the alloy is skimmed and poured to molds.

The quantity of beryllium oxide used may vary within considerable range, but I have found that as small a quantity as  $\frac{1}{25}$  of 1% is effective in promoting a perfectly homogeneous combination of the metals in almost any proportion, and which in actual practice has been remelted a half dozen times without showing a tendency to separate or stratify. As a practical matter  $\frac{1}{10}$ th of 1% by weight of the beryllium oxide to the weight of the combined metals used may

be relied upon to produce the desired homogeneity, though several times this quantity may be used.

I have also tried metallic beryllium in place of the oxide with somewhat similar results except that the resulting alloy was objectionably hard for bearing purposes.

While I have shown the value of beryllium oxide with simple copper-lead alloys it has equal value in the presence of other metals frequently introduced into copper-lead bearing alloys such as nickel used to change the physical attribute of the resulting metal, the effect of nickel additions being to increase the tensile strength.

Having thus described my improved process of making a copper-lead alloy, or alloy containing copper together with a high percentage of lead, what I claim is:

1. The process of making an homogeneous copper-lead alloy of high lead content which comprises melting the metals with the addition of a relatively small quantity of beryllium ranging between about  $\frac{1}{25}$  of 1% to about 2% by weight of the combined metals.

2. The process of making an homogeneous copper-lead alloy containing upward of 25% lead which comprises melting the metals with the addition of a quantity up to about 2% of beryllium oxide.

3. The process of making an homogeneous alloy containing copper and lead with the latter in excess of 25% which comprises melting the metals in the presence of a relatively small quantity of beryllium oxide ranging between about  $\frac{1}{25}$  of 1% to about 2% by weight of the combined metals while avoiding oxidation of the surface of the melt.

FREDERICK A. KORMANN.

90

95

100